

P.P. Meyer,  
Making Metal Vessels,  
No 60,770, Patented Jan. 1, 1867.



Witnesses.

A. Williamson  
Thos. Weston

Inventor.

Philip P. Meyer  
By. How & Weston  
Attest

# United States Patent Office.

PHILIP P. MEYER, OF NEW YORK, N. Y.

*Letters Patent No. 60,770, dated January 1, 1867.*

## IMPROVED METHOD OF MAKING SHEET-METAL VESSELS OF TWO THICKNESSES.

The Schedule referred to in these Letters Patent and making part of the same.

Specification of an improved Method of Working Metals, invented by PHILIP P. MEYER, of the city, county, and State of New York.

The object of my invention is to form vessels of two or more kinds of metals, put together in such a manner that the least corrosive metal of which the inside of a vessel is formed, as tin, for example, and which is usually the most expensive, shall be of sufficient thickness, and be strengthened by a coarser and cheaper metal or metals applied over or around it. It consists in first spinning on a chuck of suitable form a coating of tin or other incorrosive metal of any desired thickness, and then spinning on over the said coating another coating of lead, copper, or other cheaper metal, to strengthen, stiffen, and protect the interior metal, in the manner and for the purpose hereinafter set forth.

In order to give additional strength or stiffness to these metals, rings or bars of iron, steel, or other metal may be put on after the inner coating is spun on, and the outer coating of metal spun over the whole. This method is principally useful in making vessels which are destined to contain acids or other substances which would be deteriorated by coming into contact with lead, copper, iron, and other of the more corrosive metals, which vessels are commonly lined with a thin coating of tin, which, however, quickly wears off and leaves the metal underneath exposed. By my process the tin or other metal with which the vessel is lined may be made of any thickness desired, so that it may be made very much more durable. Vessels for preparing articles of food, such as the inner vessels of ice-cream freezers, have also been made wholly of tin, which renders them too expensive to permit them to come into common use, while by my process the expense is much less. In the accompanying drawings—

Figure 1 is a side elevation of a small vessel of lead and tin made by my improved process.

Figure 2 is a vertical central section of the same.

Figure 3 is a side elevation of a small vessel of copper and tin.

Figure 4 is a vertical central section of the same.

A, fig. 2, is the inner coating of tin. It is taken in a soft state and spun on over a chuck having the form of the interior of the vessel which it is intended to make. B are wires of iron or other stiff metal which are fastened to the outside of the lining A. C is a coating of lead which is then spun on over the lining A and the wires B. This lead can be spun down to the coating A, so as to make a perfect contact between them, but if it is found that the contact is not perfect, it can very easily be made so by inserting the vessel in a suitable hollow chuck and opening the lining out to meet the said coating C. D, fig. 4, is the lining of tin, and E the covering of copper of a vessel very commonly used in chemical laboratories. In place of tin, the lining may be made of silver, gold, or other metal when the vessel is to contain the more powerful acids, &c.

Other vessels of any shape desired may be made in this way by providing chucks of suitable shape on which to spin them; it being necessary, of course, when the neck or top of a vessel is of smaller diameter than some parts of its body, to provide a chuck which may be removed in pieces. Vessels or other hollow articles may be made by spinning the outside into a hollow chuck, and then, having formed the lining of nearly the proper shape on the outside of a solid chuck, by spinning the lining into the covering. Should it be desired, a coating of tin may also be spun on over the covering, which gives strength to the vessel, which would be desirable in case the vessel was destined to have its outside brought in contact with the acid or other corroding substance.

I am aware that attempts have been made to form vessels of tin and other cheaper metals, combined by forming sheets of the two vessels rolled together or joined by casting a coating of lead over tin and then spinning a vessel out of the resulting sheet of metal. I am also aware that vessels of various shapes have been made by spinning up various metals. These I do not claim.

I claim—

1. The process described for forming a vessel of two or more metals by spinning them one upon the other, for the purpose set forth.
2. The combination with a vessel constructed of two or more metals spun together as set forth, of strengthening bars or rings, substantially as herein set forth.

PHILIP P. MEYER.

Witnesses:

M. F. GUAGHTY,  
H. JAMES WESTON.